

# United States Patent

D'Alessandro

[15] 3,685,005

[45] Aug. 15, 1972

[54] **HERMETICALLY SEALED CONNECTOR**

[72] Inventor: **Franklin M. D'Alessandro, Chicago, Ill.**

[73] Assignee: **The Bunker-Ramo Corporation, Oak Brook, Ill.**

[22] Filed: **July 22, 1969**

[21] Appl. No.: **843,644**

[52] U.S. Cl. .... **339/136, 339/218, 339/278**

[51] Int. Cl. .... **H01r 13/40**

[58] Field of Search.... **174/152, 51.01, 51.61, 51.56, 174/51.55; 339/64, 144 T, 126 R, 136, 94, 278 C, 218**

[56] **References Cited**

UNITED STATES PATENTS

|           |         |                      |           |
|-----------|---------|----------------------|-----------|
| 2,674,645 | 4/1954  | Fine.....            | 339/94    |
| 2,904,456 | 9/1959  | Nolte.....           | 117/212   |
| 3,076,954 | 2/1963  | Stanback.....        | 339/278 X |
| 3,109,054 | 10/1963 | Kuhnafel et al. .... | 174/152   |

|           |         |                    |             |
|-----------|---------|--------------------|-------------|
| 3,225,132 | 12/1965 | Baas et al.....    | 174/50.61 X |
| 3,370,874 | 2/1968  | Scherer et al..... | 174/50.61 X |
| 3,371,413 | 3/1968  | Rundle .....       | 339/177 X   |

OTHER PUBLICATIONS

Electrical Manufacturing, article by J. Comer Vol. 62 No. 2 Aug. 1958 Pages 102- 107

Primary Examiner—Richard E. Moore  
Attorney—Frederick M. Arbuckle

[57] **ABSTRACT**

A hermetically sealed electrical connector capable of operation in temperatures from -55° to 225° C. As disclosed, it comprises an outer shell of light weight aluminum alloy, surrounding copper contacts extending through a glass insulator supported within the shell; the shell, the insulator, and the contacts being made from materials having specified coefficients of thermal expansion and yield strength effective to avoid destruction of the integrity of the seal by thermal expansion and contraction.

7 Claims, 2 Drawing Figures



PATENTED AUG 15 1972

3,685,005

FIG. 1



FIG. 2



INVENTOR  
FRANKLIN M. DALESSANDRO

BY  
*L. J. Hammond*  
ATTY.

## HERMETICALLY SEALED CONNECTOR

## BACKGROUND OF THE INVENTION

The invention relates generally to electrical connectors, and particularly to hermetically sealed connectors suitable for service in temperature environments ranging from very low to very high temperatures, yet light enough for use in aircraft and aerospace applications and capable for meeting certain military specifications for such use.

Hermetic electrical connectors generally employ two types of glass to metal seals, namely, a matched seal and a compression seal. With the matched seal, the metal and glass components exhibit similar coefficients of thermal expansion thereby preventing the development of excessive strains and undesirable stresses when the metal and glass contract and expand due to changes in temperature. This arrangement requires a chemical bond to be formed between the glass and metal to provide the seal.

The compression seal arrangement provides a seal between the glass and metal by a compressive force. It is desirable that a chemical bond also exist, but it is not necessary for this type of seal. The compressive force is exerted on an internal glass member by an outer metal shell having a relatively high coefficient of thermal expansion. After heating the glass and shell to a fusing temperature, the shell contracts during a cooling process to provide the compressive force on the glass member.

At this juncture it should be noted that glasses are very strong in compression and very weak in tension, and that a compression seal is possible only with an external metal member disposed about an internal glass member, whereas a matched seal can be accomplished with either an externally disposed metal member or an internally disposed metal member, i.e., a metal contact located in a surrounding glass body or member. Electrical connectors generally employ both types of seal arrangements since each connector necessarily has an external member, namely, a outer shell or housing structure and internally disposed metal members, namely, electrical contacts supported in an insulating glass body.

Hermetic electrical connectors presently available generally use, as the shell material, low carbon steels, stainless steels and other alloys having low coefficients of thermal expansion as compared to other metals. The internal glass insulators or bodies generally have even lower coefficients of thermal expansion, the values being on the order of  $9 \times 10^{-6}/^{\circ}\text{C}$ . Since the glasses used have low expansion coefficients, the material of the connector contacts are similarly limited to low expansion, special purpose alloys necessary to provide a matched seal between the contacts and glass. The most common of these are the iron-nickel alloys though tungsten and molybdenum have been used as contact materials.

Connectors constructed with the materials described above offer adequate mechanical strength to withstand stresses developed under thermal shock conditions but are substantially heavier than the connectors of the present disclosure since the density of steel and iron alloys average as about 8g/cc as compared to 2.7g/cc for aluminum. Further, because of the high electrical resistance of low expansion alloys, heretofore generally

used as contacts, prior art hermetic connectors have been characterized by high contact resistance and thus relatively low current carrying capabilities. For example, a low expansion alloy of iron and nickel (50 percent iron and 50 percent nickel), which is a commonly used alloy for making contacts, has an electrical conductivity value of 4 percent IACS (International Annealed Copper Standard) as compared to pure copper which has a conductivity value of 101 percent IACS.

Heretofore, attempts have been made at using aluminum shells in the construction of hermetically sealed connectors. In U.S. Pat. No. 3,371,413 issued to D.F. Rundle and assigned to the present assignee, there is shown an aluminum shell structure in combination with a steel ring bonded to the periphery of a glass body. The steel ring (with the glass) is then force-fitted into the aluminum shell to form a mechanical seal between the steel and aluminum. Such a structure gains the advantage of the light weight of aluminum but the mechanical seal between the metals of the ring and shell is not as reliable as a seal provided by fusion. Further, the force fitted seal is somewhat difficult to produce in large quantities because of extremely close tolerance requirements.

Another attempt at using aluminum as the material of a connector shell has simply involved the use of an aluminum shell in combination with the known low expansion glasses and low expansion alloy contacts. While gaining the advantage of the light weight of aluminum, the low expansion glasses in such aluminum connectors subject the seal interface and the aluminum shell to severe stresses because of the substantial difference in thermal expansion between the glass and aluminum. Aluminum alloys have a coefficient of thermal expansion on the order of  $25 \times 10^{-6}/^{\circ}\text{C}$ . Further, most glasses have temperatures higher than the melting point of aluminum; most aluminum alloys melting at temperatures below 650° C., and in addition, the low expansion alloy contacts have the low electrical conductivity characteristic noted above.

Historically, the major difficulty in providing a hermetic connector in an aluminum shell has been the detrimental effect of the high coefficient of thermal expansion value of aluminum. While a high compressive force can be exerted on the inner glass body by the aluminum, when the connector cools after the firing and sealing process, a correspondingly high tensile force is exerted on the shell. This tensile force produces stresses in the shell which can exceed the yield strength of the aluminum. When this occurs, the inner diameter of the shell wall deforms plastically and enlarges, thereby reducing the compressive force on the glass to a value proportional to the yield strength of the aluminum. Upon reheating, such as may occur during service, the seal expands elastically, and the stresses are reduced. Hence at sufficiently high temperatures, the compressive force exerted by the shell on the glass is reduced to zero and further heating places the glass in tension, a mode in which it is very weak as explained above. Failure occurs when the glass breaks or separates from the shell which represents the the thermal shock limit of the connector. Thus, the connectors made with aluminum shells have heretofore been unable to withstand operating temperatures of over approximately 100° C.

It should be noted further that aluminum alloys are originally hardened by working and heat treating processes, and that most aluminum alloys suffer a decrease in their original hardness (i.e. their yield strength) when subjected to the firing process necessary for providing a connector with a hermetic seal. This firing process for providing the hermetic seal acts as an annealing process which tends to soften the aluminum of the shell. Thus, aluminum shells in the annealed condition are even less able to withstand the stresses exerted on the shell by the internal glass body.

#### BRIEF SUMMARY OF THE INVENTION

The present invention provides a hermetically sealed electrical connector which is light in weight, has high electrical conductivity, and can withstand both low and high operating temperatures; i.e. temperatures in the range of from  $-55^{\circ}\text{C}$ . (as required by some U.S. Military Specifications) to  $225^{\circ}\text{C}$ . without loss of the connector's hermeticity. This may be accomplished by using an outer shell structure made of a light weight aluminum alloy characterized by high yield strength (in an annealed or post-fired condition) and with a coefficient of thermal expansion greater than that of the glass (to provide compressive force thereon in cooling) but not so much greater than that of the glass as to permanently stretch or distort the metal of the shell and thus pre-dispose the connector to failure whenever subjected to such elevated temperatures in service.

#### THE DRAWING

The invention, along with the objects and advantages thereof, will best be understood from consideration of the following detailed description taken in connection with the accompanying drawing in which:

FIG. 1 is a sectional view of a temperature-resistant hermetically sealed connector constructed in accordance with the principles of the invention; and

FIG. 2, is a sectional view of a preformed glass insulator used in construction of the connector of FIG. I.

#### PREFERRED EMBODIMENT

Specifically, FIG. 1 shows a sectional view of a connector 10 constructed in accordance with the inventive principles presently to be disclosed. More particularly, the connector 10 includes an outer shell or housing generally designated 12 but ordinarily including a mounting flange 14 and a receptacle portion 16 to receive a mating connector. In practice, this shell may include various forms of keyways 18, grooves 20 and coupling pins 22 as shown, but these form no part of the present invention.

The shell 12 does however have a central bore 24 extending through the mounting flange 14 and in communication with the receptacle portion 16 of the shell to provide for mounting the glass insulator 26 which in turn carries at least one metallic contact 28, each of which has a terminal portion 30 disposed exteriorly of the connector and an internal pin portion 32 within the receptacle 16. The glass insulator 26 is, of course, held in position and hermetically sealed within the bore 24, being fused to the internal walls of the bore 24 and to the individual contacts 28.

The outer shell 12 is made of a light weight aluminum alloy characterized by having a relatively high yield strength (for example 15,000 pounds per square inch or preferably 21,000 pounds per square inch or more in an annealed or post-fired condition) and having a coefficient of thermal expansion well above that of the insulator 26, but within certain limits: generally not exceeding 1 and  $\frac{1}{2}$  times the coefficient of the glass.

10

5

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

258

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

15

The glass insulator 26, is preferably a pre-formed, unitary member which is formed to have the correct size and shape to fit in the bore 24 of the shell 12 and to receive the contacts 28 before it is sealed in the shell. This may be accomplished by first grinding the glass material into a powder and then placing the powder in a mold (not shown) to be pressed and pre-fired to form a single piece pre-form as shown in FIG. 2. The pre-form is provided with chamfered or bevelled peripheral edges 34 and countersunk holes 36 for receiving the contacts 28. The chamfered edges and countersunk holes promote the development of a smooth, uniformly stressed glass fillet 38 between the contact members 28 and the outer shell 12 during a firing process for providing the seals. This is indicated by the uniform cross section and rounded corners of the insulating body 26 shown in FIG. 1. Without the pre-formed chamfer and countersunk holes, the glass tends to form irregular stress risers and depressions during the firing process.

After the glass insulator 26 is pre-formed, it is inserted and suitably located within the bore 24 through the shell 12. Hermetic seals are then provided between the metal of the contact and the glass, and between the metal of the shell and the glass by a firing process which heats the glass to its working temperature. At this temperature, the glass is softened to provide an adequate glow thereof within the shell and about the contacts, the glass forming a bond with the contacts.

With the cooling of the connector, the shell contracts on the glass insulator since the metal of the shell has a greater expansion coefficient ( $23.4 \times 10^{-6}/^{\circ}\text{C.}$ ) than that of the glass which is  $17 \times 10^{-6}/^{\circ}\text{C.}$  as explained above. The difference in the expansion coefficients of the glass and shell in the present invention, however, is not as large as those of prior art devices which use low expansion glasses ( $9 \times 10^{-6}/^{\circ}\text{C.}$ ) in aluminum shells. Thus, in the present invention, the stress imposed on the shell 12 by the glass insulating body 14 is substantially lower than that of the prior art aluminum connectors. This lower stress characteristic, coupled with the high yield strength of the shell material, provides the connector of the present invention with highly reliable hermetic seals since the tendency of the shell to deform plastically is substantially reduced. In this manner, the thermal shock limit of the glass insulating body is substantially increased since the high yield strength of the shell maintains the glass in compression at operating temperatures substantially higher than heretofore possible with hermetic aluminum connectors.

Thermal shock tests were conducted on connector samples of the invention by rapidly changing the temperature of their operating environment from a low temperature value on the order of  $-55^{\circ}\text{C.}$  to a high temperature value on the order of  $225^{\circ}\text{C.}$ , and continuously operating the connectors at a minimum of  $200^{\circ}\text{C.}$  This was accomplished without the loss of hermeticity. The seals and glass thus withstood temperature extremes substantially greater than prior art aluminum which, as explained above, have a maximum operating temperature of about  $100^{\circ}\text{C.}$

In addition to the extended temperatures at which the connector of the invention will operate in a reliable manner, the connector offers a substantial weight reduction over conventional steel and iron alloy con-

nectors. This is of particular importance in the aerospace and aircraft industry where weight is a primary consideration.

Also, as heretofore explained, use of copper for the contacts provides the connector with greatly increased electrical conductivity over that of prior art connectors. In order to protect the copper of the contacts from excessive oxidation during the firing and sealing process, the contacts may be clad or plated with nickel, 10 rhodium or other suitable oxidation resistant metals.

It should now be apparent from the foregoing description that the applicant has disclosed a highly reliable, hermetically sealed electrical connector which is light in weight, has high electrical conductivity and is thermally shock resistant over a range of temperatures never achieved by prior art devices.

Having thus described the invention, I claim:

1. A hermetically sealed electrical connector capable of maintaining hermetic integrity throughout a temperature range from as low as  $-55^{\circ}\text{C.}$  up to at least  $225^{\circ}\text{C.}$  and comprising, in combination, a hollow metal shell of an aluminum alloy having an opening therethrough; the opening having side walls closely surrounding and engaging a glass insulator fused therein and in tight compression relationship therewith; with at least one electrical contact fused into said insulator and extending therethrough; said contact being of metal having a coefficient of thermal expansion matched to 20 that of said insulator and being supported solely thereby; the glass having a working point lower than the melting point of the metal shell, and the metal shell having a coefficient of thermal expansion greater than that of the glass but not more than  $1\frac{1}{2}$  times that of the glass and being characterized by a yield strength such that said glass insulator may be fused within the shell and thereafter cooled to  $-55^{\circ}\text{C.}$  without imparting strains upon the metal shell which causes stresses exceeding the annealed yield strength thereof.

2. The device of claim 1 wherein the glass has a coefficient of thermal expansion of substantially  $17 \times 10^{-6}/^{\circ}\text{C.}$  and the metal shell is an aluminum alloy.

3. The device of claim 1 wherein the metal shell is an aluminum alloy having a yield strength determined on said shell in an annealed condition of at least 15,000 pounds per square inch, and having a coefficient of thermal expansion of substantially  $23.4 \times 10^{-6}/^{\circ}\text{C.}$

4. The connector described in claim 1 in which the 50 glass insulator is a unitary, pre-formed member having the peripheral edges thereof chamfered, and at least one countersunk hole for accommodating the contact, the chamfered edges and countersunk hold providing uniformly stressed fillets between the glass and the shell and between the contact and the glass.

5. A hermetically sealed electrical connector capable of maintaining hermetic integrity throughout a temperature range from as low as  $-55^{\circ}\text{C.}$  up to at least  $225^{\circ}\text{C.}$  and comprising, in combination a hollow aluminum alloy shell having an opening therethrough; the opening having side walls closely surrounding and engaging a glass insulator fused therein and in tight compression relationship therewith; with at least one copper electrical contact extending through the insulator and fused into said insulator and supported solely thereby; the glass having a working point lower than the melting point of the shell and substantially  $540^{\circ}\text{C.}$

and having a coefficient of thermal expansion of substantially  $17 \times 10^{-6}/^{\circ}\text{C}$ . and the metal shell having a coefficient of thermal expansion of substantially  $23.4 \times 10^{-6}/^{\circ}\text{C}$ . and being characterized by a yield strength determined on the said aluminum shell in an annealed condition of at least 15,000 pounds per square inch so that said glass insulator may be fused within the shell and thereafter cooled to  $-55^{\circ}\text{C}$ . without imparting strains upon the shell which cause stresses exceeding the said yield strength thereof.

6. The device of claim 5 wherein the yield strength of the shell determined on the shell in an annealed condi-

tion is at least 21,000 pounds per square inch and the aluminum alloy is the aluminum alloy designated as 5083 Aluminum by the U.S.A Standards Institute.

7. The connector described in claim 6 in which the glass insulator is a unitary, pre-formed member having the peripheral edges thereof chamfered and at least one countersunk hole for accommodating a contact; the chamfered edges and countersunk hole providing uniformly stressed fillets between the glass and the shell and between the contact and the glass when the connector is subjected to a firing temperature.

\* \* \* \* \*

15

20

25

30

35

40

45

50

55

60

65